

B. W. ELDER.

PROCESS FOR PRODUCING CATALYZERS FOR HYDROGENATION.

APPLICATION FILED JUNE 7, 1918.

1,331,904.

Patented Feb. 24, 1920.



Inventor  
BENJAMIN W. ELDER

By

Attorney

Charles A. Teller

# UNITED STATES PATENT OFFICE.

BENJAMIN W. ELDER, OF LOS ANGELES, CALIFORNIA, ASSIGNOR TO THE ALLBRIGHT-  
NELL COMPANY, A CORPORATION OF ILLINOIS.

## PROCESS FOR PRODUCING CATALYZERS FOR HYDROGENATION.

1,331,904.

Specification of Letters Patent.

Patented Feb. 24, 1920.

Application filed June 7, 1918. Serial No. 238,655.

To all whom it may concern:

Be it known that I, BENJAMIN W. ELDER, a citizen of the United States, and a resident of the city of Los Angeles, in the county of 5 Los Angeles and State of California, have invented certain new and useful Improvements in Processes for Producing Catalysts for Hydrogenation; and I do hereby declare that the following is a full, clear, and exact 10 description of the same, reference being had to the accompanying drawings, and to the numerals of reference marked thereon, which form a part of this specification.

This invention relates to an improved 15 method of producing finely pulverulent catalysts, and more particularly finely pulverulent nickel catalysts, adapted for use in the catalytic hydrogenation of oils and of other unsaturated substances.

20 The invention is based upon the discovery that nickel, in bulk form, which possesses practically no catalytic activity, can be converted into a finely pulverulent nickel catalyst which is highly catalytic by subjecting 25 the bulk nickel to a mechanical grinding or attrition or abrading operation in an apparatus of the type commonly known as a tumbler or ball mill, or pebble mill. As a result of the operation to which the bulk 30 nickel is subjected, there is developed in the nickel a high degree of catalytic activity which renders the resulting finely pulverulent catalyst well adapted for use for various purposes, and particularly for use in 35 the catalytic hydrogenation of unsaturated fatty bodies such as the unsaturated fatty acids and their glycerids or esters.

I have further ascertained that the treatment of the bulk nickel, and the conversion 40 of the bulk nickel into an active catalyst, can be effected with particular advantage, in an apparatus of the character referred to, with the added use of a finely divided abrasive which is free from anti-catalytic properties, and which will be present at the end 45 of the operation in intimate intermixture with the finely pulverulent nickel catalyst produced.

The bulk nickel which is utilized in the 50 process of the present invention, may be any suitable or convenient form of nickel which possesses practically no catalytic activity, and which is free from constituents prejudicial to the development in the nickel of the 55 desired catalytic properties. As such forms

of nickel may be mentioned nickel shot, or nickel in lump form, or turnings, clippings, or other forms of nickel adapted and available for use for the production of an active nickel catalyst.

60 The invention will be further described and illustrated in connection with the accompanying drawing illustrative of one of the forms of apparatus adapted to the practice of the process of the present invention.

In the accompanying drawing there is illustrated in longitudinal vertical section and with parts in elevation, a tumbler or pebble mill, 1, of circular or polygonal shape, mounted in a frame 2, which is journaled in 70 upright bearing standards 3 and capable of being rotated by a pulley 4 secured upon an extension of the frame. The bulk nickel, preferably grain nickel, is introduced into the tumbler through a suitable opening (not 75 shown), or by the removal of one end of the tumbler as 5. Extending into one end of the drum, through one end of the bearing frame 2, is an inlet pipe 6, and extending into the other end thereof in a similar manner is an 80 inlet pipe 7.

The bulk nickel, in any suitable form, may be introduced into the tumbler or pebble mill, either alone or together with a finely divided abrasive. When no abrasive is used, 85 the nickel slot or other form of bulk nickel will, during the rotation of the tumbler, be subjected to attrition or abrasion, and the bulk nickel will be gradually converted into finely divided nickel particles. This operation may be carried out at ordinary 90 temperatures, and frequently without extra precautions, although it is sometimes advantageous, and may even be desirable, to protect the nickel against oxidation during the operation.

95 This may be effected by the introduction of a non-oxidizing gas, such as hydrogen, through the pipe 6, or by the introduction of a protective liquid, such as oil, through the pipe 7; or by the introduction 100 of both a protective gas and a protective liquid. When the protective liquid is an unsaturated oil, and the protective gas is hydrogen, some catalytic hydrogenation of the oil may be brought about during the production of the catalyst, and particularly if the temperature is raised to such a temperature as will materially promote the catalytic hydrogenation process.

105 When an abrasive is used, it may be added

either in small amount or in large amount. When added in small amount, the nickel shot or other nickel particles will still be brought into abrasive relation with each other, and the abrasive action will be promoted by the intervening finely divided abrasive. When larger amounts of abrasive are used, the nickel shot or other nickel particles may be entirely separated from each other so that the action is essentially an action of the abrasive upon the nickel particles. When an abrasive is used, a protective liquid, such as oil, or a protective gas, such as hydrogen, may be also employed in the manner above described.

During the rotation of the tumbler or pebble mill, the bulk nickel will be subjected to a rubbing or grinding or abrasive action, with resulting attrition or grinding or abrasion of the bulk nickel, and with accompanying development in the resulting finely divided nickel of a high degree of catalytic activity. The operation is preferably carried on under such conditions and for such a time that the nickel will be brought into a finely pulverulent state readily adapted to be maintained in suspension in a liquid medium, as, for instance, in the fatty acid or its ester to be hydrogenated; but as the development of the catalytically active condition of the material seems to be in part at least a function of the attrition incident to the operation, it is not absolutely necessary that the material, or all of the material, should be brought into a finely pulverulent form. It may, in some instances, in part at least, have a different physical form than that of fine powder, provided always that the operation has been carried on under such conditions and for such a time as to develop and maintain in the ultimate particles the desired catalytic activity.

Where the nickel employed in bulk form is metallic nickel, the catalyst produced will similarly be of a metallic character, substantially free from oxygen and oxides which are always present in catalysts produced by the incomplete reduction with hydrogen of nickel oxid or similar reducible nickel compounds.

The abrasive, when used, is preferably of a finely pulverulent character. I have thus found abrasives of about 200 mesh as well adapted for use in the process of the present invention. The finely divided abrasive should be free from anti-catalytic properties and from constituents prejudicial to the development of the desired catalytic activity. Among the available abrasives may be mentioned silica, quartz, alundum, emery, carbondum, etc.

Where an abrasive is used, the finely pulverulent product resulting from the operation will contain the finely divided abrasive in intimate admixture with the finely pul-

verulent catalyst. This composite product, containing the catalyst particles and the abrasive, is available for use, without separation of the abrasive, for catalytic purposes, inasmuch as the finely divided abrasive will not usually be prejudicial, and may even be advantageous in the carrying out of the catalytic process.

Where a protective liquid, such as oil, is present during the operation, there will result at the end of the operation a more or less thick oil mud containing the finely divided abrasive and the finely divided catalyst particles in suspension in the oil. It will be evident that varying amounts of oil can be used as well as varying amounts of abrasive, and that the resulting product will correspondingly vary in its oil and abrasive content, and in its content of finely divided catalyst particles. During the tumbling or pebble mill operation the minute particles of the nickel separated from the bulk nickel will be enveloped by the oil and maintained in suspension therein and carried thereby. These particles will also be thereby protected from contact with the air which may be present within the tumbler or pebble mill.

The amount of finely divided catalyst particles will increase with the prolongation of the ball mill operation. The fineness or minuteness of the particles produced will also tend to increase with prolongation of the operation, inasmuch as the fine particles first produced will be further subjected to the attrition or abrasive action during the further continuation of the operation. It is readily possible, when using a finely divided abrasive, or even without such an abrasive, to produce an exceedingly finely divided nickel catalyst of a sufficient degree of fineness so that it can be readily maintained in suspension in liquids, for example, fatty oils, for considerable periods of time and with but slow settling out therefrom. The particles tend to approach colloidal particles in fineness or size. Such a finely divided catalyst is well adapted for use in the catalytic hydrogenation of oils and can be readily maintained in suspension therein.

In many cases the finely divided abrasive will be of a different order of fineness from the finely divided catalyst particles produced, and will tend to settle out at a different rate. In such cases, it is possible to effect a partial separation of the finely divided catalyst and of the finely divided abrasive, for example, by differential sedimentation, so that the catalyst may be available with a less content of abrasive, and so that the abrasive may be available, if desired, for further use in the production of further amounts of finely divided catalyst.

In the operation of the tumbler or pebble

mill, and particularly where this is not operated too slowly, there will take place a combined rubbing, squeezing and percussive action, of the lumps or particles of bulk nickel upon each other, either with or without the added action of the abrasive. This combined rubbing, squeezing and percussive action is particularly well adapted for the development of the desired catalytic properties in the bulk nickel and the production therefrom of a finely pulverulent catalyzer.

The particular type and construction of the tumbler or pebble mill, can be varied, as will be evident. So also, the charge of bulk nickel, which it will contain, will vary with its size; and the amount of finely pulverulent nickel catalyzer produced will also vary with the length of prolongation of the operation. When the operation has been continued a sufficient time, with the resulting development and production of a sufficient amount of highly active pulverulent catalyzer, the operation can be stopped and the catalyzer withdrawn. Any remaining bulk nickel may be left in the apparatus for the next operation, and further amounts of bulk nickel may be added thereto together with further amounts of abrasive and protective liquids such as oil, etc. The operation can be then repeated in substantially the manner above described.

From the foregoing description it will be evident that the process of the present invention is one of marked simplicity, requiring a minimum of attention and supervision. The ball mill operation, once started, may be allowed to continue without attention for long periods of time, until the operation has progressed sufficiently to give the desired amount of catalyzer, in the desired state of subdivision and catalytic activity.

As compared with the processes of the prior art involving the reduction of reducible nickel compounds with hydrogen at an elevated temperature, it will be noted that the present process enables the chemical methods of solution and precipitation, for converting bulk nickel into a reducible nickel compound, to be done away with; and also enables the furnace operation, for reducing the reducible nickel compound and producing the reduced nickel catalyzer, to be done away with; and that the present process not only eliminates these elaborate and expensive chemical operations, but enables a finely divided catalyzer, of high catalytic activity, to be produced directly, in metallic form, from the raw metallic nickel, possessing practically no catalytic activity.

The product produced according to the present invention is moreover distinguished from finely divided catalysts produced by reduction with hydrogen at elevated tem-

peratures of reducible nickel compounds in that it is essentially metallic in character, when produced from raw metallic nickel, and in that its particles, although they may be of microscopic size, are nevertheless characteristic of the mechanical operation by which they are produced.

When produced in the presence of oil, the product will be a more or less thick mud containing the catalyzer particles, either with or without the finely divided abrasive.

Having thus described my invention what I claim is:

1. The method of producing a catalyzer, which comprises subjecting substantially non-catalytic catalyzer material to a combined rubbing, squeezing and percussive action, and thereby producing a finely pulverulent catalyzer of high catalytic activity.

2. The method of producing a catalyzer, which comprises subjecting catalyzer material to a ball mill operation in admixture with a finely-divided abrasive, and thereby producing a finely pulverulent catalyzer in admixture with the abrasive.

3. The method of producing a catalyzer, which comprises subjecting the catalyzer material to a ball mill operation in the presence of a protective liquid and thereby producing a finely pulverulent catalyzer in suspension in said liquid.

4. The method of producing a catalyzer, which comprises subjecting catalyzer material, in admixture with a finely-divided abrasive and a protective liquid, to a ball mill operation, and thereby producing a finely pulverulent catalyzer in suspension in said liquid and in admixture with the finely pulverulent abrasive.

5. The method of producing a catalyzer, which comprises subjecting substantially non-catalytic bulk nickel to a ball mill operation, and thereby producing a finely pulverulent nickel catalyzer of high catalytic activity.

6. The method of producing a catalyzer, which comprises subjecting substantially non-catalytic nickel to a combined rubbing, squeezing and percussive action, and thereby producing a finely pulverulent nickel catalyzer of high catalytic activity.

7. The method of producing a catalyzer, which comprises subjecting bulk nickel to a ball mill operation in admixture with a finely divided abrasive, and thereby producing a finely pulverulent nickel catalyzer in admixture with the abrasive.

8. The method of producing a catalyzer, which comprises subjecting bulk nickel to a ball mill operation in the presence of a protective liquid and thereby producing a finely pulverulent nickel catalyzer in suspension in said liquid.

9. The method of producing a catalyzer,

which comprises subjecting bulk nickel, in admixture with a finely divided abrasive and a protective liquid, to a ball mill operation, and thereby producing a finely pulverulent nickel catalyzer in suspension in said liquid and in admixture with the finely pulverulent abrasive.

10. The method of producing a catalyzer, which comprises subjecting the bulk nickel to a ball mill operation in the presence of a fatty oil and thereby producing a finely pulverulent nickel catalyzer in suspension in said oil.

11. The method of producing a catalyzer,

which comprises subjecting bulk nickel, in admixture with a finely divided abrasive and a fatty oil, to a ball mill operation, and thereby producing a finely pulverulent nickel catalyzer in suspension in the oil and in admixture with the finely pulverulent abrasive.

In testimony whereof I have hereunto subscribed my name in the presence of two subscribing witnesses.

BENJAMIN W. ELDER.

Witnesses:

A. WIGHTMAN,  
F. N. CLAFLIN.